

Patented Feb. 9, 1926.

1,572,490

## UNITED STATES PATENT OFFICE.

RODERICK L. JOHNSTON, OF PLAINFIELD, NEW JERSEY, ROBERT S. ARCHER, OF LAKEWOOD, AND ZAY JEFFRIES, OF SHAKER HEIGHTS, OHIO, ASSIGNEES TO ALUMINUM COMPANY OF AMERICA, OF PITTSBURGH, PENNSYLVANIA, A CORPORATION OF PENNSYLVANIA.

### ALUMINUM ALLOY.

No Drawing. Original application filed November 27, 1920, Serial No. 426,793. Divided and this application filed February 11, 1925. Serial No. 8,517.

To all whom it may concern:

Be it known that we, RODERICK L. JOHNSTON, of Plainfield, county of Union, and State of New Jersey, ROBERT S. ARCHER, of 5 Lakewood, and ZAY JEFFRIES, of Shaker Heights, both in the county of Cuyahoga and State of Ohio, all citizens of the United States of America, have invented certain new and useful Improvements in Aluminum 10 Alloys, of which the following is a full, clear, and exact description.

The presence of small amounts of silicon in aluminum and in aluminum alloys is usually considered objectionable. In the 15 course of an investigation upon the effects of silicon we have discovered that by using a substantial amount of silicon, materially greater than the quantity usually found as an impurity, with the addition of a metal 20 or metals, for example one or more of those hereinafter named, it is possible to produce an alloy having excellent casting qualities combined with good physical properties.

Among the metals capable of forming 25 solid solutions in the aluminum we have found copper and zinc particularly advantageous. The metals referred to may be used singly or in combination. In the use of copper alone, the silicon content of the 30 alloy should in general be not less than about 3 per cent nor more than about 10 per cent, and the copper should be preferably from about 2 per cent to about 5 per cent; the proportions of copper and silicon 35 being variable, however, according to the particular combination of properties desired. In general, the attainment of good casting qualities depends largely upon the relative proportions of the silicon and 40 copper, the latter being preferably reduced as the former is increased, and vice versa. Increasing the copper, at least up to the limit of its capacity for entering into solid solution in the aluminum, tends in general 45 to increase the tensile strength, especially if subjected to a suitable heat treatment, say that described in Patent No. 1,508,556, issued September 16, 1924, to Zay Jeffries and Robert S. Archer. A test bar cast in 50 sand in the ordinary way, of an aluminum alloy containing 10 per cent silicon and 3 per cent copper, showed a tensile strength

of about 23,000 pounds per square inch and an elongation of about 1.5 per cent in two inches. Such a bar, after heat treatment by 55 the method described in the above mentioned patent, showed an increase of tensile strength up to 30,000 pounds per square inch and an increase of elongation up to 2.5 per cent. A bar of the same alloy but 60 cast in a chill mold, in order to cause rapid solidification of the molten metal, was found to have a tensile strength of about 30,000 pounds per square inch and an elongation of about 2.7 per cent, even without 65 heat treatment. A similar bar, heat treated, had a tensile strength of 40,000 pounds per square inch and 6 per cent elongation. On the other hand, a chill-cast heat-treated bar of an alloy containing about 6 per cent 70 silicon and about 4 per cent copper was found to have a tensile strength exceeding 42,000 pounds per square inch and an elongation exceeding 8 per cent in 2 inches. Alloys of aluminum, silicon and copper are 75 described and claimed in our copending application identified hereinafter.

The addition of zinc up to about 5 per cent has a slight effect on the tensile strength of the alloy. Above that amount 80 a greater increase of tensile strength is observed. The presence of the zinc is often an advantage by reason of the whiter color of the polished alloy. We have found that with the addition of an alkali metal or 85 metals to the alloy, as described in patent of Junius D. Edwards, Francis C. Frary and Harry V. Churchill, No. 1,410,461, issued March 21, 1922, very satisfactory physical properties can be obtained along 90 with the other advantages incident to the presence of the zinc, particularly if the alloy to which alkali metal has been added is cast in such a manner, as for example by the use of a chill mold, that the molten 95 metal is caused to solidify rapidly. For instance, an alloy containing about 10 per cent zinc and about 8 per cent silicon, to which alkali metal had been added and which was cast in a chill mold, has been 100 found to have a tensile strength exceeding 42,000 pounds per square inch, with an elongation up to 7 per cent in two inches. A similar casting, after being subjected to

the heat treatment described in the above mentioned patent of Archer and Jeffries, showed a decrease of tensile strength to about 35,000 pounds per square inch, but 5 an increase of elongation up to 14 per cent.

In the case of aluminum-silicon alloys containing both copper and zinc, a sand cast test bar of an alloy containing 8 per cent silicon, 10 per cent zinc and 2.5 per 10 cent copper, was found to have a tensile strength of 27,000 pounds per square inch and an elongation of 1.5 per cent. This alloy is also susceptible to improvement by addition of alkali metal before casting; 15 sand cast specimens of the alloy so treated having a tensile strength of 30,000 pounds per square inch with an elongation of 2 per cent, while chill cast specimens have a tensile strength of 38,000 pounds per square 20 inch and an elongation of 3.5 per cent. Heat treatment by the method described in the patent of Archer and Jeffries before referred to has been found to increase the tensile strength of the chill cast alloy up 25 to 45,000 pounds per square inch and at the same time increase the elongation to 7.5 per cent.

In the alloys referred to above we have observed that the elongation is better if 30 the iron content is low, and for that reason there are many cases where the iron should not exceed about 0.6 per cent. In other cases much higher iron can be used, especially in chill castings, as for example 35 sure die castings.

The alloys described herein are also well adapted to forging and like operations.

While in certain of the claims certain percentages and limits have been stated it is 40 to be understood that they may be somewhat departed from without departing from the

invention sought to be protected, so long as the properties of the alloy are retained.

This application is a division of our co-pending application, Serial No. 426,793, filed November 27, 1920.

We claim:

1. An alloy composed chiefly of aluminum, containing, approximately, silicon 8 per cent, zinc 10 per cent, and copper 2.5 per cent. 50

2. An alloy composed chiefly of aluminum, containing silicon between 3 and 10 per cent, and zinc, the latter not exceeding about 15 per cent. 55

3. An alloy composed chiefly of aluminum, containing silicon between 3 and 10 per cent, and zinc between 5 and 15 per cent, approximately.

4. An alloy composed chiefly of aluminum, containing about 8 per cent silicon, and about 10 per cent zinc. 60

5. An alloy composed chiefly of aluminum, containing, approximately, silicon 8 per cent, zinc 10 per cent, and copper 2.5 per cent, with an iron content not exceeding about 0.6 per cent. 65

6. An alloy composed chiefly of aluminum, containing silicon between 3 and 10 per cent and zinc, the latter not exceeding about 15 per cent, with an iron content not exceeding about 0.6 per cent. 70

7. An alloy composed chiefly of aluminum, containing about 8 per cent silicon and about 10 per cent zinc, with an iron content not exceeding about 0.6 per cent. 75

In testimony whereof we hereto affix our signatures.

RODERICK L. JOHNSTON.  
ROBERT S. ARCHER.  
ZAY JEFFRIES.